# EUROPEAN PATENT SPECIFICATION

(11) **EP 2 406 406 B1**
(45) Date of publication and mention of the grant of the patent: **22.11.2017**
(21) Application number: 09841636.5
(22) Date of filing: 12.08.2009
(51) Int. Cl.: C22C 38/58

(54) **LEAD-FREE BRASS ALLOY**
BLEIFREIE MESSINGLEGIERUNG
ALLIAGE DE LAITON SANS PLOMB

(30) Priority: 09.03.2009 US 400283
(43) Date of publication of application: 18.01.2012
(73) Proprietor: National Bronze & Metals, Inc., Houston, TX 77008-6113 (US)
(72) Inventor: LAZARUS, Norman, Michael, Houston TX 77024 (US)
(74) Representative: J A Kemp
(86) International application number: PCT/US2009/053505
(87) International publication number: WO 2010/104527

(56) References cited:
- CN-A- 1 563 449
- JP-A- S6 274 037
- JP-A- H04 128 332
- US-A1- 2009 016 927
- US-B1- 6 471 792

## Description

### TECHNICAL FIELD

The present invention relates to brass compositions with extremely low to no lead content. The compositions exhibit good machinability and strength similar to that of conventional leaded brass alloy free machining brass.

### BACKGROUND OF THE INVENTION

It has been common practice to add up to 4.5% lead to brass compositions to improve the machinability of the resulting product. Lead, however, is a toxic substance and its use in the production of alloys is surrounded by legislation and expensive control procedures. For example, California adopted legislation which limits the amount of lead in plumbing fixtures to .25% or less beginning in 2010.

Furthermore, the lead phase in copper lead alloys can be affected by corrosive attacks with hot organic or mineral oil. For example, when temperature of such an alloy rises, it has been known that the oil can break down to form peroxides and organic gases which effect a degree of leaching on the lead phase within the alloy. If this leaching progresses to any appreciable extent, the component, if it is a bearing or structural component, may eventually malfunction or fail.

There is, therefore, considerable advantage in reducing, or if possible, eliminating the contents of lead within powder metallurgy compositions. Various proposals have been put forward for doing this. The considerable proportions of lead incorporated in powder metallurgy materials in the past has resulted in ease of machinability and durability of the resulting product component. Replacement of part of the lead by bismuth has been proposed in International Application published under No. WO91/14012. This results in successful replacement of part of the lead without significant reduction in the machinability. It is, however, accompanied by some reduction of transverse strength of the material. For many purposes this reduction in transverse strength is not a significant problem.

Another approach has been described in U.S. Patent 5,445,665. In this product 0.1 to 1.5% graphite is added to the alloy allowing for reduction of lead to 2% of the alloy or less. The Japanese patent JP 4-128332 discloses a brass alloy containing 25-38% Zn together with 0.005-0.5% Te that offers excellent resistance to dezinctification as well as improved corrosion resistance.

While the alloys described above yield substantially lead-free alloys, they do not possess the same machinability as the lead containing alloys. This results in the need for substantial retooling of the equipment used to produce end product, such as plumbing equipment and the like. In addition, the scrap produced during the manufacturing of the lead products often cannot be readily recycled by the end product manufacturer. Recycling typically can only be done by the manufacturer of the alloys. The cost of shipping the scrap back to the initial foundry increases the overall product cost of the end product.

Thus, there remains a need for a lead-free brass alloy which exhibits machinability similar to that of lead containing products and that can be recycled by the customer.

### BRIEF SUMMARY OF THE INVENTION

The present invention relates to a brass alloy consisting of: copper, from 2% to less than 15% zinc, from 0.4% to 1.0% tellurium, less than 0.25% lead, and optionally less than 0.02% phosphorus. The alloy typically has a lead content of from less than 0.025% to less than 0.001% which is considered "lead-free."

The alloy exhibits excellent machinability and conductivity. Depending on the composition of the alloy, the tensile strength will vary between 240 MPa and 530 MPa and yield strength will vary from 200 to 450 MPa. Conductivity will range from 28% to 49% IACS. The machinability of the novel alloy of the invention is similar to that for lead containing compositions. This eliminates or reduces the amount of retooling needed to use the novel alloys to produce finished products such as plumbing fixtures.

The composition of the novel alloy also allows the end product manufacturers to recycle the scrap from the manufacturing process itself. This eliminates the need to return the scrap to the alloy manufacturer for recycling. Yet another key feature of the present invention is that the alloy, which contains less than 15% zinc, exhibits excellent dezincification resistance.

### BRIEF DESCRIPTION OF THE DRAWINGS

Figure 1 is a photomicrograph of the alloy used in Sample C1 after draw.
Figure 2 is a photomicrograph of the alloy used in Sample C2 after draw.
Figure 3 is a photomicrograph of the alloy used in Sample C3 after draw.

### DETAILED DESCRIPTION OF THE INVENTION

The brass alloys of the present invention are prepared by first melting copper at a temperature of about 1050°C. Zinc and tellurium are then added to the molten copper. Brass alloy is then cast into billets utilizing horizontal or vertical casting methods.

The copper used to make the alloys is typically copper cathode or high grade uncontaminated and pure copper scrap comprising 99.95% minimum copper and to .05% impurities. Lead is a typical impurity, comprising less than 0.025% of the copper used.

Zinc is the next major component comprising from 2% to less than 15% of the alloy.

Tellurium is used as a replacement for lead. Like lead, tellurium is added to improve machinability of the alloy without the negative contribution of lead. Tellurium is added in an amount ranging from 0.4% to 1.0%. In one embodiment, tellurium comprises about .5% of the alloy. The amount of tellurium used will depend, in part, on the amount of copper used in the alloy, as copper levels increase the amount of tellurium used with decrease. Like lead, the addition of tellurium to the alloy creates discontinuities in the copper and zinc phases of the alloy like those shown in Figs 1-3. The good dispersion of these discontinuities leads to the improved machinability of the alloys.

One advantage of the present invention is that the alloys exhibit machinability similar to that of lead containing alloys while using significantly lower amounts of tellurium.

Other materials which may be added to the brass alloys include phosphorous. When phosphorous is used, the amount present will typically be less than 0.02% of the alloy.

The resulting alloys will generally exhibit excellent machinability and conductivity as indicated by Ultimate Tensile Strength (UTS) ranging from 240 to 530 MPa and a yield strength of from 200 MPa to 450 MPa as determined using ASTM method B140. The actual Tensile strength and Yield strength will depend, in part, on the actual composition of the alloy. Conductivity of the alloys will range from 28 to 45% IACS.

### EXAMPLES

A series of brass alloys were prepared where the added lead (typically about 2%) was replaced with approximately 0.5% tellurium. The composition of each alloy is shown in Table 1 (Samples C and D do not fall within the scope of protection).

| TABLE 1 | | | | | | |
|---|---|---|---|---|---|---|
| Sample | Cu | Pb | Zn | Te | P | Sn |
| A | Balance | <0.01 | 5.10 | 0.5 | 0.011 | ---- |
| B | Balance | 0.00 | 8.82 | 0.57 | .001 | ---- |
| C | 83.03 | 0.06 | Balance | .052 | 0.05 | 0.11 |
| D | 59.41 | 0.02 | Balance | 0.17 | 0.05 | ---- |

The billets were then changed into an extrusion press at a temperature ranging from about 780°C to about 860°C. The billets were then hot extruded through a variety of dies and at different pressures to produce numerous sizes. Each shot was lubricated prior to extrusion and the extrusion dies were preheated. The results are shown in Table 2.

| **TABLE 2** | | | | |
|---|---|---|---|---|
| Sample | Final Draw Size | Shot Temp | Pressure | Length |
| A1 | 31.75mm | 808°C | 234MPa | 12m |
| A2 | 75.40mm | 822°C | 268MPa | 18.5m |
| A3 | 19.05mm | 803°C | 305MPa | 34m |
| B1 | 31.75mm | 794°C | 267MPa | 12m |
| B2 | 25.40mm | 800°C | 289MPa | 18.5m |
| B3 | 19.05mm | 806°C | 304MPa | 34m |
| B4 | 12.70mm | 870°C | 265MPa | 67m |
| C1a | 25.40mm | 830°C | 298MPa | 18.4m |
| C1b | 25.40mm | 867°C | 280MPa | 18.4m |
| C2a | 50.80mm | 750°C | 230MPa | 21.5m |
| C3a | 22.23mm AF Hex | 830°C | 312MPa | 21.5m |
| C3b | 22.23mm AF Hex | 837°C | 324MPa | 21.5m |
| D1a | 50.8mm | 640°C | 128MPa | 4.6m |
| D1b | 50.80mm | 637°C | 142MPa | 4.6m |
| D2a | 25.4mm | 650°C | 234MPa | 18.4m |
| D2b | 25.4mm | 660°C | 214MPa | 18.4m |
| D3a | 22.23mm AF Hex | 648°C | 235MPa | 21.5m |
| D3b | 22.23mm | 621°C | 276MPa | 21.5m |

The bars were then passed through a bath of sulfuric pickling acid and then cold drawn so as to induce the correct mechanical properties and grain size requirements. Also this process ensures that the correct size tolerances are met. The cold drawing operation was accomplished effortlessly. The products were then tested for tensile strength, hardness, conductivity, and machinability. The results are shown in Table 3.

| **TABLE 3** | | | | | |
|---|---|---|---|---|---|
| **Sample** | **Reduction in Area (%)** | **Ultimate Tensile Strength (MPa)** | **Yield Strength (MPa)** | **ELONGATION** | **HARDNESS (Rb)** |
| A1 | 11.24 | 267.9 | 210.3 | 30% | 56 |
| A2 | 12.8 | 296.5 | 341.3 | 24% | 57 |
| A3 | 1_.71 | 322 | 279.2 | 16% | 60 |
| B1 | 11.24 | 302.7 | 241.3 | 26% | 59 |
| B2 | 12.8 | 322 | 259.2 | 24% | 63 |
| B3 | 17.71 | 322.7 | 268.9 | 21% | 64 |
| B4 | 28.32 | 393.7 | 393 | 12% | 69 |
| C1 | 12.8 | 350.2 | 291.9 | 20% | 51 |
| C2 | 11.13 | 354.9 | 295.8 | 20% | 52 |
| C3 | 13 | 358.8 | 294.1 | 22% | 53 |
| D1 | 14.10 | 487.8 | 378.2 | 29% | 75 |
| D2 | 14.10 | 531.6 | 443 | 20% | 78 |
| D3 | 14.44 | 485.3 | 407.8 | 19% | 76 |

Conductivity tests were then conducted on various samples. Conductivity diminishes as the ratio of zinc content increases. The results ranged from at least about 28% to about 49% maximum.

Photomicrographs of Samples C1, C2 and C3 were taken after draw and are shown in FIGS 1-3. The micro structure in the alloys were uniform indicating good dispersion of the tellurium throughout the alloy.

## Claims

1. A brass alloy consisting of:
copper;
from 2% to less than 15% zinc;
from 0.4 % to 1.0% tellurium;
less than 0.25% lead; and
optionally less than 0.02% phosphorous.

2. The alloy of claim 1 having a lead content of less than 0.025%.

3. The alloy of claim 1 having a lead content of less than 0.001%.

4. The alloy of claim 1 having a tensile strength of from 240MPa to 530MPa.

5. The alloy of claim 1 having a yield strength of from 200MPa to 450MPa.

6. The alloy of claim 1 having a conductivity of from 28% to 49% IACS.

## Patentansprüche

1. Messinglegierung bestehend aus:
Kupfer;
von 2 % bis weniger als 15 % Zink;
von 0,4 % bis 1,0 % Tellur;
weniger als 0,25 % Blei; und
optional weniger als 0,02 % Phosphor.

2. Legierung nach Anspruch 1 mit einem Bleigehalt von weniger als 0,025 %.

3. Legierung nach Anspruch 1 mit einem Bleigehalt von weniger als 0,001 %.

4. Legierung nach Anspruch 1 mit einer Zugfestigkeit von 240 MPa bis 530 MPa.

5. Legierung nach Anspruch 1 mit einer Streckfestigkeit von 200 MPa bis 450 MPa.

6. Legierung nach Anspruch 1 mit einer Leitfähigkeit von 28 % bis 49 % IACS.

## Revendications

1. Alliage de laiton composé de :
cuivre ;
de 2 % à moins de 15 % de zinc ;
de 0,4 % à 1,0 % de tellure ;
moins de 0,25 % de plomb ; et
éventuellement moins de 0,02 % de phosphore.

2. Alliage selon la revendication 1 ayant une teneur en plomb inférieure à 0,025 %.

3. Alliage selon la revendication 1 ayant une teneur en plomb inférieure à 0,001 %.

4. Alliage selon la revendication 1 ayant une résistance à la traction allant de 240 MPa à 530 MPa.

5. Alliage selon la revendication 1 ayant une limite d'élasticité allant de 200 MPa à 450 MPa.

6. Alliage selon la revendication 1 ayant une conductivité allant de 28 % à 49 % IACS.
